

Aug. 10, 1926.

1,595,454

D. M. CRIST

PROCESS OF METALLIZING FINE ORE CONCENTRATES

Filed Dec. 26, 1924

2 Sheets-Sheet 1



Fig. 1



Fig. 2

INVENTOR

D. M. CRIST

BY *Wright & Chriss*

ATTYS

Aug. 10, 1926.

1,595,454

D. M. CRIST

## PROCESS OF METALLIZING FINE ORE CONCENTRATES

Filed Dec. 26, 1924

2 Sheets-Sheet 2



*INVENTOR*  
*J.M. CRIST*

BY *Wright & Dunn*  
ATTYS

Patented Aug. 10, 1926.

1,595,454

# UNITED STATES PATENT OFFICE.

DONALD M. CRIST, OF SAN FRANCISCO, CALIFORNIA, ASSIGNOR TO TRIUMPH STEEL CO., OF RENO, NEVADA, A CORPORATION OF NEVADA.

## PROCESS OF METALLIZING FINE ORE CONCENTRATES.

Application filed December 26, 1924. Serial No. 758,017.

The present invention relates to the art of reducing fine ore concentrates and resides in the provision of a process and an apparatus by means of which fine ore concentrates may 5 be more rapidly, thoroughly and economically reduced than is possible under other methods and with other apparatus, and also without necessitating briquetting of the ore.

One of the objects of the invention is to 10 provide a comparatively simple and inexpensive apparatus for carrying out this invention, which apparatus may be operated efficaciously and at a low cost.

A further object of the invention is to provide 15 for treatment of fine ore concentrates so as to bring about a rapid and thorough reduction without melting the ores.

Another object of the invention is to provide 20 for the use of gases generated in the treatment of the ores under this invention, for heating ores or operating apparatus with which the process or method is carried out.

With the above mentioned and other objects in view, the invention consists in the 25 novel construction and combination of parts hereinafter described, illustrated in the accompanying drawings, and set forth in the claims hereto appended, it being understood that various changes in the form, proportion, 30 size and minor details of construction within the scope of the claims may be resorted to without departing from the spirit or sacrificing any of the advantages of the invention.

35 Referring to the drawings:

Fig. 1 represents a longitudinal sectional view taken through apparatus constructed in accordance with the present invention.

Fig. 2 is a sectional view taken on line 40 2-2 of Fig. 1.

Fig. 3 represents a fragmentary longitudinal sectional view being shown partly in elevation of a modified form of the apparatus constructed in accordance with the invention.

Fig. 4 represents a sectional view taken on line 4-4 of Fig. 3.

In carrying out the process of this invention, ore to be treated is passed through a 50 zone heated to disassociation temperature for the particular ore, and is subjected to this heat for a period of time sufficient to thoroughly break down the ore without fusion, the said zone being shut off from communication with atmospheric air. This

treatment of ore will bring about a rapid, thorough reduction. In the treatment of certain ore a catalyzing or reducing agent is introduced into the heated zone to carry away the volatiles liberated in the treatment. 60 This agent is preferably of a carbonaceous nature and will produce a gas which may be burned in the fire-box to heat the zone or otherwise utilized to produce power for the operation of the apparatus of the invention. 65

Referring to the embodiment of the invention shown in the accompanying drawings (Figs. 1 and 2), the apparatus with which the process of the invention is carried out comprises a suitable furnace generally 70 designated 1, having the usual fire-box 2, provided at one end with an outlet flue 3, and at its other end with an ore discharge passage 4, which latter is arranged to discharge ore into a water jacketed hopper 5 75 having a closure valve 6 at its lower end, which valve is operated by a suitable gear 7. Adjacent one end of the furnace supported in suitable frame work 8, is a hopper 9 for containing ore to be treated. The ore is arranged to pass through a heated zone extending through the furnace, which zone is in communication with the passage 4 so as to discharge the reduced ore into the hopper 5. 80 This zone is provided in the form of a revolvable cylinder 10 mounted on suitable bearings 11 within the furnace and having one end extending into an open end of the passage 4 and provided with a suitably packed gland 12 so as to provide an air 85 tight seal at this point. The other end of the tube extends out through one wall of the furnace and is rotatably coupled by suitable means 13 with a stationary pipe or conduit 14. This pipe 13 extends downwardly 90 from this connection with the cylinder and then horizontally to a point where it communicates with the firebox 2 so that gases generated in the treatment of the ores as will be later described, will be delivered to the 95 firebox for consumption to assist in heating the cylinder.

A valved feed chute 15 extends from the hopper 9 into the pipe 14 close to the point where the joint 13 is provided so as to convey ores into the pipe or conduit, and from thence into the cylinder 10. The pipe and cylinder are inclined downwardly from the point where the chute 15 enters the pipe 14 100 so that the ores will gravitate through the 105 cylinder. The pipe 14 is inclined downwardly from the point where the chute 15 enters the pipe 14 so that the ores will gravitate through the 110 cylinder.

cylinder into the discharge passage 4. The interior of the cylinder is provided with a plurality of longitudinally extending feed ribs 16, each of angular construction and rigidly arranged within the cylinder. These ribs serve as a means for guiding and conveying the ores through the cylinder during the rotation of the latter. A gear 17 is fastened to the outer end of the cylinder and is driven by a gear 18, which latter is operated by any suitable source of power, not shown.

As shown in Fig. 1 there is provided a means for introducing a catalyzing or reducing agent into the lower or discharge end of the cylinder 10. This means comprises a tank or container 19 in which fuel oil, crude oil, or some other carbonaceous fuel, the present instance of liquid form, will be contained. From the container or hopper 19 a downwardly curved feed pipe 20 extends, said pipe being provided with a control valve 21 near its upper end. This pipe extends through the adjacent end wall of the furnace and well into the lower end of the cylinder so as to be spaced from the walls of the latter. A water jacket 22 surrounds the pipe so as to keep it cool and may be supplied with water from any suitable source, not shown.

In the operation of the invention fine ore concentrates are fed from the hopper 9 through the discharge chute 15 into the heated zone or in other words, cylinder 10, said cylinder being operated so as to revolve. The fire-box is provided with a suitable burner, not shown, so as to heat the cylinder sufficiently to produce a suitable ore disassociation temperature interiorly thereof, this temperature varying depending on the ore being treated. The cylinder is rotated at such speed and is at such an inclination that the ore will be caused to remain in it for a period of time just sufficient to thoroughly bread it down. The angular ribs extending longitudinally of the cylinder assist in retarding and agitating the ores so as to bring about the desired treatment during the passage of the ores through the cylinder. This treatment is carried out in a zone from which free air is excluded, and the ores break down and are deoxidized without being melted, the reduced ore passing out of the cylinder through the passage 4 into the water-cooled hopper 5. From this the treated ore may be taken off as desired, upon manipulation of the valve 6.

In the case of certain ores, oil or other carbonaceous material is fed into the heated cylinder through the pipe 20 and acts as a catalyzing or reducing agent to carry off the volatiles liberated during treatment of the ores. The carbonaceous material thus used will generate a gas which will pass through the pipe 14 and into the fire-box where it

may be ignited for the purpose of assisting in the heating of the cylinder.

In Figs. 3 and 4, the apparatus shown is adapted for the use of carbonaceous material such as coal dust, as a reducing or catalyzing agent, and the cylinder is electrically heated by an element contained in the cylinder. Although a fire-box is not shown in connection with this type of furnace, it is obvious that this might be used instead of the electric heating arrangement.

In this form, the apparatus comprises a cylinder 23, rotatably mounted in position slightly inclined from the horizontal, on suitable supports 24. The upper end of the cylinder is connected by a stuffing box or gland, generally designated 25, with a pipe 26, which latter extends to a gas container or bell 26 mounted on a platform 28. An ore feed hopper 29 is supported on this platform and has a valve discharge chute 30 which extends into the pipe adjacent to the joint 25. A gear 31 is fixed to the upper end of the cylinder and meshes with a gear 32 mounted on a shaft 33 journaled in the support 24. This shaft is coupled to a shaft 34 driven from a suitable source of power and which through a train of gears 35, rotates a feed screw 36 in a feed pipe 37 extending into the lower end of the cylinder. The lower end of the cylinder is mounted in a wall member 38 which is provided with a conduit or discharge 39, into one end of which discharge said cylinder extends and is rotatably mounted. A suitable gland 40 provides for an air tight seal between the passage 40 and said cylinder. Supported by this wall, by a standard 41 extending adjacent to it, is a container or hopper 42 for carbonaceous material such as coal dust. The lower end of the hopper has a discharge chute 43 which communicates with the feed pipe 37. Thus, on rotation of the shaft 34, that is required to rotate the cylinder 23, through the gears 32 and 33, the train of gears operate to rotate the feed screw 36 and for feeding the carbonaceous material through the pipe 37 into the cylinder 23. The passage or conduit 39 discharges into a water-jacketed container or hopper 44 adapted to receive the reduced ores. This hopper or container closes at its lower end by a valve 45 and an operating means 46. The cylinder 23 is of special construction to adapt it for being heated by electricity. Interiorly of the cylinder is a lining of refractory material 47 having a suitable heating element 48 embedded therein. This lining protects the cylinder from being burned out by the heating element, causes the interior of the cylinder to be thoroughly heated to the temperature necessary to carry out the treatment of this invention. The terminals of the heating element are electrically connected with contact rings 49 on the exterior

of the casing adjacent the lower end thereof. These rings are engaged by brushes 50 which are connected with a source of electrical energy by conductors 51, said brushes being supported by a bracket 52 carried by the wall 38.

The operation of this form of the invention is the same as in the preferred form except that gases generated are carried off 10 through the pipe 26 into bell or container 27 and this stored up gas may be used for the purpose of generating power for operating the machinery of the apparatus.

I claim:

15 1. The process of reducing ore which consists in continuously passing ore to be treated through a zone heated to a disassociation temperature, causing said ore to remain at said temperature in said zone for a sufficient period of time to thoroughly break down the ore then continuously taking off the ore from said heated zone.

20 2. The process of reducing ore which consists in continuously passing ore to be treated through a zone heated to a disassociation temperature, causing said ore to remain at said temperature in said zone for a sufficient period of time to thoroughly break down the ore, then taking off the ore from said heated zone and continuously introducing, during the treatment of the ore in said zone, a carbonaceous material.

25 3. The process of reducing ore which consists in passing ore to be treated through a zone heated to a disassociation temperature, causing said ore to remain at said temperature in said zone for a sufficient period of time to thoroughly break down the ore, then taking off the ore from said heated zone and continuously introducing, during the treatment of the ore in said zone, a carbonaceous material.

time to thoroughly break down the ore, then taking off the ore from said heated zone and introducing, during the treatment of the 40 ore in said zone, a carbonaceous material and taking off the gases generated in the treatment of the ore.

4. The process of metallizing ore which consists in passing ore to be treated through 45 a zone heated to a disassociation temperature, causing the ore to continuously pass through said zone, introducing carbonaceous matter into the zone and taking off gases generated in the treatment and igniting said 50 gases to heat said zone.

5. The process of metallizing ore which consists in continuously passing ore to be treated through a zone heated to a disassociation temperature and from which zone atmospheric air is excluded causing said ore to remain in said zone for sufficient time to cause the ore to break down without melting and without arresting the progress of the 55 ore through said zone, and continuously taking off the ore from said zone.

6. The process of metallizing ore which consists in causing ore to be continuously fed into and continuously moved through a zone heated to a disassociation temperature for 60 the particular ore, from which zone atmospheric air is excluded and in which zone said ore remains for sufficient time to cause the ore to break down without melting, then introducing carbonaceous material into the 70 zone and continuously taking off ore from said zone.

DONALD M. CRIST.